

Jan. 17, 1961

E. C. MILBERGER ET AL  
FLUID POWER TRANSMISSION

2,968,625

Filed July 25, 1956



INVENTORS.  
ERNEST C. MILBERGER &  
SAMUEL M. DARLING

BY

*Campbell, Brumbaugh, Free & Graves*  
their ATTORNEYS.

1

2,968,625

## FLUID POWER TRANSMISSION

Ernest C. Milberger, Maple Heights, and Samuel M. Darling, Lyndhurst, Ohio, assignors to The Standard Oil Company, Cleveland, Ohio, a corporation of Ohio

Filed July 25, 1956, Ser. No. 600,024

2 Claims. (Cl. 252—75)

This invention relates to fluid power transmission and to a power transmission fluid characterized by an ASTM slope below 0.3, comprising a light mineral oil of normal viscosity index, and an inorganic gelling agent and imidazoline in amounts to impart an ASTM slope of below 0.3 to the mineral oil.

Petroleum oils have certain performance characteristics which make them particularly suitable for use as power transmission fluids. A power transmission fluid which is well suited for the job for which it is intended must have good flowability and pumpability, lubricating ability, chemical stability, rust-inhibiting ability, demulsibility, and defoaming ability. All of these characteristics are important, and should be displayed over the entire range of temperatures at which the system is to be used. All fluids, however, undergo a change in viscosity with temperature. The rate of change of viscosity with change in temperature which characterizes petroleum oils is not as low as that for many synthetic oils such as silicone oils and the Ucon oils, which are polypropylene glycol ethers, and this is a disadvantage.

The rate of change in viscosity with temperature of petroleum oils ordinarily is measured by the viscosity index, usually abbreviated V.I. The higher the V.I., the lower the rate of change in viscosity, and the better the petroleum oil for use as a hydraulic fluid. However, the viscosity index loses its sensitivity as a characterizing property when the oil has an exceptionally low rate of change in viscosity, of the order of that which characterizes many synthetic oils. A viscosity temperature relationship has been developed which is superior to the viscosity index for this type of petroleum oil. This is the ASTM slope, adopted as a standard method by the American Petroleum Institute, Standard 533-43, ASTM designation D-341-43. This slope is the tangent of the acute angle of the viscosity-temperature plot of the oil on the ASTM standard chart D-341-43. The smaller the ASTM slope, the flatter the curve, and the lower the change in viscosity with temperature.

Typical ASTM slopes of a number of petroleum and synthetic oils are given below:

| Petroleum Oils                      | Viscosity, 100° F. | SSU, 210° F. | ASTM Slope |
|-------------------------------------|--------------------|--------------|------------|
| Straw Paraffin                      | 74.1               | 36.6         | 0.78       |
| Automatic Transmission Fluid        | 200                | 50           | 0.66       |
| Synthetic Oils:                     |                    |              |            |
| Silicone Oils—                      |                    |              |            |
| Dow Corning 550                     | 440                | 101          | 0.45       |
| General Electric 9981-LT-125        | 577                | 231          | 0.23       |
| Ucon Oils <sup>1</sup> —            |                    |              |            |
| LB 385                              | 385                | 75.1         | 0.55       |
| LB 525                              | 525                | 93.1         | 0.51       |
| LB 650-X                            | 650                | 106          | 0.51       |
| Esters—                             |                    |              |            |
| Bis-(2-ethylhexyl) sebacate         | 67.8               | 37           | 0.70       |
| Bis-(3,5,5-trimethylhexyl) sebacate | 94.6               | 41.3         | 0.65       |

<sup>1</sup> Monobutyl poly 1,2-oxy propylene glycols. See Kirkpatrick U.S. No. 2,615,853.

2

The lighter mineral oils of low viscosity would be especially suitable for use as power transmission media because of their low sludge and deposit-forming tendencies compared to the heavier oils. However, light oils lack lubricating ability under operating conditions, and ASTM slope is in most instances too high. In fact, the light oils have such a low viscosity at high temperatures that they are not suited without modification for such purposes.

10 In accordance with this invention, power transmission fluids are provided having a viscosity within the range from 75 to 1000 SSU at 100° F. and from 50 to 750 SSU at 210° F., and an ASTM slope below about 0.3, employing as the base oil light lubricating oils having a viscosity of about 50 to 300 SSU at 100° F. and from 25 to 55 SSU at 210° F. The ASTM slope of the light lubricating oils is not critical because the power transmission fluids of the invention nonetheless have an ASTM slope of less than 0.3, considerably less than many synthetic oils and most ordinary petroleum hydrocarbon oils, even when highly refined, as the above table shows.

15 The power transmission fluids of the invention comprise from 1 to 3% based on the weight of the oil of an inorganic gelling agent, and from about 1% to about 20% by weight of the gelling agent of an imidazoline having an aliphatic radical of from 8 to 20 carbon atoms. These two additives in combination increase the viscosity of the light oil to the point where the composition has a viscosity suitable for a power transmission fluid, and in addition improve the ASTM slope of the base oil to below 0.3. The compositions of the invention are fluid under all conditions of use at normal and elevated temperatures.

20 These effects are not obtained in the absence of either the inorganic gelling agent or the imidazoline. The increase in the viscosity and decrease in the ASTM slope due to the inorganic gelling agent are relatively small. The imidazoline alone has no effect upon viscosity or ASTM slope. However, in the presence of the inorganic gelling agent the imidazoline effects a further increase in viscosity, and a further decrease in the ASTM slope. Thus, the imidazoline makes it possible to achieve higher viscosities and lower ASTM slope within the desired ranges, using lesser amounts of the inorganic gelling agent. The viscosity-increasing and ASTM slope decreasing effects of the imidazoline are obtained after the mixture of oils, gelling agent and imidazoline has been heated to temperatures of 300° F. or higher.

25 The lubricating oil stock used in preparing the compositions of the invention will have a viscosity within the range from 50 to 300 SSU at 100° F. and 25 to 55 SSU at 210° F. The base stock is preferably a lubricating oil fraction of petroleum and it may be unrefined, acid-refined or solvent-refined, as required for the particular lubricating need. The nature of the base oil makes little difference in the relative consistencies of the compositions, although conventionally acid-refined oils produce slightly thicker fluids than the solvent-refined oils. The viscosity index of the oil is not critical.

30 The inorganic gelling agent can be any inorganic material which is dispersible in the oil and which is so finely divided as to be nonabrasive. The preferred materials are the aerogels which can be formed from any material not incompatible with the oil, such as silica, alumina and magnesia. Other gel-forming metal oxides, hydroxides and sulfides can be used, of which attapulgite, the bentonites (such as Wyoming bentonite, montmorillonites and hectorite), beidellite, saponite, nontronite, sepiolite, biotite, vermiculite and zeolites, synthetic clays such as magnesia-silica-sodium oxide, lime-silica-potassium oxide and baria-silica-lithium oxide are exemplary, as well as synthetic zeolites, of which the complex aluminum silicates are exemplary.

A series of silica aerogels which can be used as the inorganic gelling agent of the invention are manufactured by Monsanto and marketed under the trade name "Santocel."

"Santocel" C is prepared from an alkali silicate solution. Silicic acid dissolves in caustic alkali such as sodium hydroxide and the alkali silicates, such as sodium silicate, can be obtained from various natural minerals and clays or by fusing silicon dioxide with alkali hydroxides or carbonates. Fused alkali silicates such as water-glass, sodium tetrasilicate ( $Na_2Si_4O_9$ ) can be completely dissolved on long heating with water, but the result is not a solution of the silicate as such but of silicic acid peptized by alkali as well as free alkali. By addition of an acid to such a solution, for example, an inorganic acid such as sulphuric acid, hydrochloric acid or carbonic acid, or an organic acid such as acetic acid, oxalic acid or formic acid, the silicic acid is precipitated in the form of a gel which is called a hydrogel or aquogel. The structure of this gel has not been fully elucidated but it is generally accepted that it is composed of a honeycomb structure of the silicon dioxide  $SiO_2$  within the pores of which is enclosed the aqueous solution remaining after precipitation of the silicic acid. Thus, it can be generally stated that these hydrogels can be obtained starting from any water-soluble alkali silicate, including not only water glass as mentioned above but sodium metasilicate  $Na_2SiO_4$ , sodium metasilicate nonahydrate  $Na_2SiO_4 \cdot 9H_2O$  and sodium disilicate  $Na_2Si_2O_5$ . All of these silicates are soluble in water, in which they decompose to form silicic acid solution.

Such an aqueous solution of silicic acid will contain sufficient  $SiO_2$  in solution to form a hydrogel containing within the range from 3% to about 12% silica as  $SiO_2$ , after gel formation by addition of the acid. The amount of silica can readily be calculated, depending upon the amount of acid which is required to acidify the solution and whether the acid employed is concentrated or diluted. It is not necessary to characterize the silicic acid solution in terms of the alkali content calculated either as  $Na_2O$  or  $NaOH$  inasmuch as this forms a salt with the anion of the acid employed and is washed out of the aquogel at the time of alcogel formation.

After formation of the aquogel, the gel is washed free from salts and excess acid, and then converted to an alcogel by soaking in ethyl alcohol or some other water-soluble volatile aliphatic alcohol. Several portions of the alcohol may be necessary completely to remove the aqueous solution. The resulting alcogel then is placed in an autoclave. In order to remove the liquid phase without a collapse of the gel structure, the autoclave is heated at a temperature above the critical temperature of the alcohol, and the pressure is allowed to increase to a point above the critical pressure of the alcohol. The vent valve is then opened and the alcohol allowed to escape. Under these conditions the silica gel structure remains practically undisturbed and the liquid phase of the gel is replaced with air. The material is then reduced in particle size by blowing it through a series of pipes containing sharp bends with jets of compressed air. Santocel C has a secondary particle size of about three to five microns.

Santocel A is prepared as set forth for Santocel C up to the point of removal of the product from the autoclave. This material is run through a continuous heating chamber where it is heated for one-half hour to a temperature of about  $1500^{\circ} F.$  to eliminate the last traces of volatile material. It is then broken down in a reductionizer or micronizer to a particle size of about one-sixteenth inch in diameter. The  $SiO_2$  content of the original hydrogel used in preparing Santocel C is approximately 9.75%, whereas that of Santocel A is about 7.0%.

AR is a modification of A, differing only in that the material is reductionized to about the same particle size as C, approximately three to five microns in diameter.

ARD is a modification of AR, differing only in that

ARD is densified by extracting air under vacuum, and therefore has a smaller volume than AR.

AX is an A which has not been devolatilized.

CDv is a C which has been devolatilized as set forth for Santocel A. The Santocel is reductionized before being devolatilized.

CDvR differs slightly from CDv in that the CDvR has been devolatilized just after heating in the autoclave and then reductionized. It differs from CDv in that the latter is reductionized before being devolatilized.

The primary differences between the A and C series are as follows:

(1) The C's are prepared from a sodium silicate solution containing 25% more silica than the A's. Therefore, in general the A's are lighter and composed of smaller particles than the C's.

(2) The A's have undergone a devolatilization step in their preparation.

The following are the bulk densities of several of the preferred silica aerogels:

|     | Density, grams per ml. |
|-----|------------------------|
| AR  | 0.029                  |
| ARD | 0.056 to 0.064         |
| C   | 0.082                  |

In general, AR and ARD show superior gelling ability and the A's in general are better than the C's. Silica aerogels which have been devolatilized generally have a higher gelling efficiency than the undevolatilized aerogels.

Other types of inorganic gelling agents which may be used include a Fumed Silica marketed by B. F. Goodrich Company. It is finely divided and appears very much like an aerogel. It is made by combustion or vaporization process, as a source of white "carbon black" for the rubber industry. The particles are several microns in size and porous in nature.

Another material is "Linde Silica Flour" marketed by Linde Air Products Co. It is very similar in physical appearance to the silica aerogel. The particle size of the silica is purported to be 0.01 to 0.05 micron and the silica is said to be manufactured by burning silicon tetrachloride and collecting the combustion product on cool plates analogous to the production of carbon black. The particles are thought to be aggregates or clusters of particles rather than of sponge-like character.

Still another inorganic gelling agent known is "Ludox" silica from Du Pont, which is known as a silica sol, and silica derivatives thereof. It has a particle size of the order of 0.01 to 0.03 micron.

The silicas from Columbia-Southern also are useful. These have the following properties.

| 55    | Wet Screen Retained 325 Mesh, Percent | Brunauer-Emmett-Teller Nitrogen Absorption Surface Area, $m^2/gm.$ |
|-------|---------------------------------------|--------------------------------------------------------------------|
| 0.004 |                                       | 257.0                                                              |
| 0.01  |                                       | 236.5                                                              |
| 0.02  |                                       | ca. 210.0                                                          |
| 0.008 |                                       | 215.5                                                              |
| 0.004 |                                       | 228.0                                                              |

65 In preparing the compositions of the invention it is necessary to remove the water from the sol and replace it with an oil. This is possible by formulating the sol and removing the water by flash distillation or azeotropic distillation.

No attempt is made to enumerate all of the inorganic gelling agents which will be suitable nor to present examples of all of them since the novel aspects of the invention reside in the composition prepared by combining them with the oil in a combination with an aliphatic amine rather than the use of novel gelling agents per se.

The imidazoline employed in the compositions of the invention has the following general structure:



where R is hydrogen, alkyl or a hydroxy alkyl radical having from 1 to 18 carbon atoms and R' is an alkyl or alkylene group having from 8 to 20 carbon atoms.

These compounds are prepared by reaction of aliphatic acids and diamines followed by cyclization, in the following way:



where  $R$  and  $R'$  are the same as in the general formula.

Illustrative R' radicals are undecyl, tridecyl, pentadecyl, undecenyl, heptadecyl and heptadecenyl. Illustrative R radicals are ethyl, methyl, propyl, butyl, hexyl, hydroxyethyl, hydroxyisopropyl, hydroxybutyl and hydroxyhexyl.

The imidazoline should be oil-dispersible or oil-soluble and will also be hydrophobic in view of the long-chain aliphatic group at the R' position.

The relative proportions of the inorganic gelling agent and the oil will vary somewhat depending upon the desired viscosity in the final composition, the gelling ability of the inorganic gelling agent and viscosity of the oil used. Compositions made with the lower viscosity oils require a somewhat larger amount of inorganic gelling agent to give a composition of the same viscosity. The compositions of the invention are fluids. In general, the amount of inorganic gelling agent falls within the range of from 1 to 3% and in most cases preferably would be from 2 to 3%.

The viscosity as might be expected increases in a fairly linear relationship with increase in concentration of the inorganic gelling agent and the amount of gelling agent can be selected in relation to the desired viscosity in view of this.

The concentration of the imidazoline usually will lie within the range from about 1% to about 20%, preferably from 5 to 10%, based on the weight of the inorganic gelling agent, but here again the amount employed will depend upon the increase in stability without an excessive increase in viscosity, the desired amount and nature of the gelling agent and the economics involved. A cheaper compound can of course be used in much larger quantities than an expensive compound at the same total cost as the lubricant.

The composition is made simply by mixing the inorganic gelling agent, the oil and the imidazoline in any order or manner. The imidazoline also can be incorporated with the inorganic gelling agent before mixing with the oil, for example, by dissolving the imidazoline in a solvent such as pentane, mixing it with the gelling agent and then evaporating the pentane. Such a treating agent can be sold as an article of commerce and dispersed in an oil when the composition of the invention is to be prepared.

Generally, the imidazoline is dispersed in the oil and the inorganic gelling agent added thereto and mixed therewith. Any simple mixing technique can be employed and if desired the mixture can be homogenized in a colloid mill.

The imidazoline must be uniformly distributed in the composition or on the inorganic gelling agent and for this reason the imidazoline is oil-dispersible or oil-soluble or else soluble in some medium in which it can be applied to the gelling agent before incorporating the latter in the oil.

The composition of the invention is not limited to the 75

oil, gelling agent and imidazoline. Any of the materials conventionally added to lubricants can be included. The expression "consisting essentially of" as used herein is intended to refer to the components which are essential to the composition, that is, the oil, the inorganic gelling agent and the imidazoline, and the expression does not exclude other components from the composition which do not render it unsuitable as a hydraulic fluid.

The following examples illustrate preferred embodiments of the invention:

### *Examples 1 to 5*

15 Into 87.2 g. of straw paraffin oil (API gravity 60° F.,  
31.4, viscosity 74.1 SSU at 100° F., 36.6 SSU at 210° F.)  
15 ASTM slope=0.78) was dissolved 0.087 g. of Amine O  
(1- $\beta$ -hydroxyethyl-2-heptadecenyl imidazoline) and into  
this mixture was stirred 0.87 g. of Santocel AR. Additional  
compositions were prepared using 0.261 g.,  
0.348 g., 0.435 g. and 0.87 g., respectively of the Amine  
20 O. The stabilities of these dispersions were observed by  
allowing small amounts of the freshly prepared samples  
to stand in stoppered containers at room temperature  
for 24 hours with the following results:

| 25 | Example No. | Percent Imidazoline | Percent Settling |
|----|-------------|---------------------|------------------|
|    | Control     | None                |                  |
|    | 1           | 10                  | 100.             |
|    | 2           | 30                  | 6.               |
|    | 3           | 40                  |                  |
|    | 4           | 50                  |                  |
| 30 | 5           | 100                 | Hard cake.       |

35 A great increase in stability over the control is noted with an Amine O content of 10% based on the amount of the Santocel. Samples containing 30, 40, 50 and 100% of the Amine O settled to a hard cake on standing. This shows these amounts of Amine O are excessive.

### Examples 6 and 7

40 A second series of compositions was prepared containing 2.5% by weight Santocel AR in the straw paraffin oil of Examples 1 to 5. One of these samples contained 10% by weight based on the Santocel (0.25% by weight of the oil) of Amine O. After mixing the samples  
45 were subjected to high shear and temperature by recycling through a small gear pump and through a steel coil at 400° F. After this treatment, the samples were subjected to further high shear conditions by atomisation through a diesel injector nozzle set at 2500 to 3000  
50 p.s.i.g. Oil was ejected from the nozzle into a flask and held under partial vacuum to remove entrained air.

The viscosities of these samples were determined in a Stormer viscometer and compared with the viscosity of the base oil:

| Example No. | Percent Santocel | Percent Amine O | Viscosity, SSU at 100° F. | ASTM Slope |
|-------------|------------------|-----------------|---------------------------|------------|
| 30 Base     | None             | None            | 78                        | 0.78       |
| 6           | 2.5              | None            | 270                       |            |
| 7           | 2.5              | 10              | 360                       | 0.07       |

The data shows that the imidazoline increases the viscosity of the suspension. An oil with a very low ASTM slope is obtained as shown in the drawing which compares the ASTM slope of the oil containing 10% Amine O with the straw paraffin oil. The curve of a 133 V.I. oil is included for comparison; its ASTM slope is 0.66.

0 Settling tests were run on the samples which had been cycled through the gear pump, and subsequently atomised through the diesel nozzle. The atomisation was found to reduce settling to zero.

All parts and percentages in the specification and claims are by weight. Amounts of the imidazoline are by

weight of the inorganic gelling agent unless otherwise indicated. Amounts of the inorganic gelling agent are by weight of the oil.

We claim:

1. In a process for fluid power transmission the improvement which comprises transmitting power by means of a fluid having a viscosity within the range from 75 to 1000 SSU at 100° F., and from 50 to 750 SSU at 210° F., and having an ASTM slope below about 0.3, consisting essentially of a mineral lubricating oil having a viscosity within the range from 50 to 300 SSU at 100° F. and from 25 to 55 SSU at 210° F., a silica aerogel in an amount within the range from about 1% to about 3% imparting an increased viscosity and a decreased ASTM slope to the oil, and from about 1% to about 20% by weight of the silica aerogel of an aliphatic imidazoline having the following formula:



where R is selected from the group consisting of hydrogen, alkyl and hydroxylalkyl radicals having from one to eighteen carbon atoms and R' is selected from the group consisting of alkyl and alkylene radicals having from eight to twenty carbon atoms, the imidazoline imparting a further increase in viscosity and a further decrease in ASTM slope, supplementing the effect of the silica aerogel.

2. A process in accordance with claim 1 in which the  
10 imidazoline is 1- $\beta$ -hydroxyethyl-2-heptadecenyl imid-  
azoline.

**References Cited in the file of this patent**

UNITED STATES PATENTS

|    |           |               |       |               |
|----|-----------|---------------|-------|---------------|
| 15 | 2,531,440 | Jordan        | ----- | Nov. 28, 1950 |
|    | 2,554,222 | Stross        | ----- | May 22, 1951  |
|    | 2,655,476 | Hughes et al. | ----- | Oct. 13, 1953 |
|    | 2,711,393 | Hughes et al. | ----- | June 21, 1955 |
|    | 2,766,205 | Marshall      | ----- | Oct. 9, 1956  |